

# United States Patent

[11] 3,554,552

[72] Inventors **Thomas E. Nixon;**  
John A. Barber; Floyd B. Nagle, Midland,  
Mich.  
[21] Appl. No. **711,509**  
[22] Filed **Mar. 8, 1968**  
[45] Patented **Jan. 12, 1971**  
[73] Assignee **The Dow Chemical Company**  
Midland, Mich.  
a corporation of Delaware

[54] **FRANGIBLE ARTICLE COMPOSED OF**  
**POLYSTYRENE AND POLYETHYLENE WAXES**  
8 Claims, No Drawings

[52] U.S. Cl. .... **273/105.4,**  
..... **260/28.5**  
[51] Int. Cl. .... **F41j 9/16,**  
..... **C08c 11/70; C08f 45/52**

[50] **Field of Search**..... **272/56.6ss;**  
**273/105.4, 105.5, (Styrene Digest), (Ethylene**  
**Digest); 260/28.5A, (Inquired)**

[56] **References Cited**

UNITED STATES PATENTS

|           |         |                     |               |
|-----------|---------|---------------------|---------------|
| 2,353,228 | 7/1944  | Ducca .....         | 260/28.5X     |
| 3,224,984 | 12/1965 | Roper et al. ....   | 260/28.5X     |
| 3,271,119 | 9/1966  | Woodberry .....     | (273/Styrene) |
| 3,355,404 | 11/1967 | Ruffing et al. .... | 260/23S       |

*Primary Examiner*—Anton O. Oechsle

*Assistant Examiner*—Marvin Siskind

*Attorneys*—Griswold & Burdick and Richard G. Waterman

**ABSTRACT:** The invention comprises fragile molded articles composed of compositions of polystyrene and polyethylene waxes, together with a lubricant or mold release agent, which articles are useful as targets in the practice of skeet shooting.

**FRANGIBLE ARTICLE COMPOSED OF POLYSTYRENE  
AND POLYETHYLENE WAXES**

This invention concerns fragile molded articles composed of low molecular weight polystyrene and polyethylene waxes, together with a lubricant or mold release agent, which fragile articles are suitable for use as targets in practice shooting.

It has now been found that compositions of low molecular weight polystyrene and polyethylene waxes, together with a small amount of a fatty acid sufficient to act as lubricant and mold release agent, can readily be compression or injection molded to make fragile articles suitable for use in practice shooting.

More specifically, the compositions consist essentially of from 96.7 to 99.4 percent by weight of the polystyrene, from 0.5 to 3.0 percent by weight of the polyethylene wax and from 0.1 to 0.3 percent by weight of a fatty acid having from 12 to 26 carbon atoms in the molecule.

The polystyrene to be employed can have a molecular weight corresponding to a viscosity characteristic of from about 12 to about 30, preferably from 15 to 25, centipoise as determined for a 30 weight percent solution of the polystyrene in toluene at 25°C.

The polyethylene wax can be a polyethylene having a molecular weight of from about 2,000 to 4,000. Such polyethylenes have (Brookfield) viscosities of from about 2,000 to 6,000 centipoise at 250°F. 121°C.)

The fatty acid can be an aliphatic monocarboxylic acid having from 12 to 26 carbon atoms in the molecule. Among suitable fatty acids are lauric acid, myristic acid, palmitic acid, stearic acid, arachidic acid, behenic acid, lignoceric acid and cerotic acid. Mixtures of two or more of said fatty acids can also be used. The fatty acids are preferably saturated aliphatic acids, but monoethylenically unsaturated fatty acids such as dodecylenic, palmitic, oleic, ricinoleic, petroselinic, vaccenic, linoleic, linolenic, eleostearic, licanic, parinaric, taric, gadoleic, arachidonic, cetooleic, erucic or selacholeic, acid or mixtures thereof with one another or with the aforementioned saturated fatty acids can also be used.

The ingredients can be blended together in any usual way. For example, the polystyrene in granular or powdered form, the polyethylene in particulate or in finely powdered form and the fatty acid, can be dry blended by tumbling a mixture of the ingredients in the desired proportions in a suitable binder. The mixture of ingredients can be dry blended, compounded or mixed on compounding rolls, a Banbury mixer or in a plastics extruder.

In a preferred practice the ingredients are dry blended and fed to a plastics extruder wherein the materials are heated, pressed and mechanically worked and blended into a uniform product which is then extruded and is cooled and cut to a granular form suitable for molding.

In molding the compositions either the dry blended or the melt blended mixture of ingredients is employed to compression, injection, or screw injection mold said material into articles suitable for a desired purpose, e.g. as discs or as half sphere shells which are usually glued together to form balls suitable for use as targets in practice shooting. It may be mentioned that for use as targets two half sphere shells are adhered together by adhesive or solvent softening of the edges to form spheres.

The walls of the moldings suitable for use as targets in practice shooting usually have a thickness of from about 0.01 to 0.03 inch, although somewhat greater or lesser wall thickness of the moldings can be used to make fragile targets.

Small amounts of dyes, coloring agents, pigments and the like can be incorporated into the compositions to make molded articles prepared therefrom more visible, are not required.

The following example illustrates ways in which the principle of the invention has been applied but is not to be construed as limiting its scope.

**EXAMPLE**

- 5 A charge of 97.75 parts by weight of granular low molecular weight polystyrene having a viscosity characteristic of 20.5 centipoise as determined for a 30 weight percent solution of the polystyrene in toluene at 25°C. and which polystyrene had a weight average molecular weight  $M_w$  of about 45,000 and a number average molecular weight  $M_n$  of about 12,700 and 2 parts of "EPOLENE," (a waxlike polyethylene having a molecular weight of about 2,500), together with 0.25 part of powdered stearic acid, was dry blended, then was fed to a plastics extruder wherein the ingredients were heated, melted and blended into a uniform composition and were extruded, cooled and cut or broken to a granular form. Portions of the product were compression molded at a temperature of about 150°C. and 500 pounds per square inch pressure to form half sphere shells  $2\frac{1}{2}$  inches in diameter having walls 0.025 inch thick. The molded half sphere shells were easily removed from the mold without sticking or breakage. Two molded half shell spheres were solvent welded to form a sphere. The spheres were fragile objects, easily broken by dropping on the floor or by other impact. Test specimens of the spheres were shot with No. 12 (mustard seed) shot shells fired from a 22 caliber smooth bore gun and were found to readily shatter into a great plurality of pieces upon being hit. The fragile plastic spheres were useful targets for practice of indoors shooting with pellets and fine shot.
- 10 In contrast, a similar formulation prepared from low molecular weight polystyrene having a viscosity characteristic of 34.6 centipoise and an  $M_w$  of about 61,500 and a  $M_n$  of about 21,000 was unsatisfactory.
- 15 We claim:
- 20 1. A fragile article of manufacture comprising a molding having walls between 0.01 and 0.03 inch thick, prepared from a composition consisting essentially of from 96.7 to 99.4 percent by weight of polystyrene having a viscosity characteristic of from 12 to 30 centipoise as determined for a 30 weight percent solution of said polystyrene in toluene at 25°C., from 0.5 to 3 percent by weight of a polyethylene having a viscosity between 2,000 and 6,000 centipoise at 121°C., and from 0.01 to 0.03 percent by weight of an aliphatic monocarboxylic acid having from 12 to 26 carbon atoms in the molecule.
- 25 2. An article as claimed in claim 1 containing an orange dye.
- 30 3. An article as claimed in claim 1 when in the form of a disc.
- 35 4. An article as claimed in claim 1 when in the form of a hollow sphere.
- 40 5. An article of manufacture suitable for use as a target in practice and competition shooting comprising a fragile hollow sphere having walls between 0.01 and 0.03 inch thick prepared by molding half sphere shells from a composition consisting essentially of from 96.7 to 99.4 percent by weight of polystyrene having a viscosity characteristic of from 10 to 30 centipoise as determined for a 30 weight percent solution of said polystyrene in toluene at 25°C., from 0.5 to 3 percent by weight of a polyethylene having a viscosity between 2,000 and 6,000 centipoise at 121°C. and from 0.01 to 0.03 percent by weight of an aliphatic monocarboxylic acid having from 12 to 26 carbon atoms in the molecule, and adhesively forming two half sphere shells to one another.
- 45 6. An article as claimed in claim 5 containing an orange dye.
- 50 7. An article as claimed in claim 5 wherein the aliphatic monocarboxylic acid is stearic acid.
- 55 8. An article as claimed in claim 5 wherein the aliphatic monocarboxylic acid is behenic acid.